

Nov. 28, 1950

J. J. GEOGHEGAN  
PROCESS FOR MAKING FLUORESCENT SCREENS, INCLUDING  
THE ELIMINATION OF COPPER IMPURITIES

2,531,618

Filed Oct. 12, 1948



FIG. 2.

INVENTOR.  
JOHN J. GEOGHEGAN  
BY

Brown, Dank & Synnestvedt  
AGENTS

## UNITED STATES PATENT OFFICE

2,531,618

## PROCESS FOR MAKING FLUORESCENT SCREENS, INCLUDING THE ELIMINATION OF COPPER IMPURITIES

John J. Geoghegan, Philadelphia, Pa., assignor to Philco Corporation, Philadelphia, Pa., a corporation of Pennsylvania

Application October 12, 1948, Serial No. 54,081

11 Claims. (Cl. 252—301.6)

1

This invention relates to a process of making fluorescent substances used in electrical discharge devices, and is especially concerned with the making of fluorescent screens of the type used in television cathode ray tubes.

The primary object of my invention resides in the provision of a novel, simple and reliable manufacturing process which, when practiced, results in a fluorescent substance which will emit substantially white light, in response to electrical excitation.

The general requirements for fluorescent screens have been described in the art, and such screens usually have consisted of mixtures of two or more fluorescent materials. For example, a zinc sulfide phosphor which fluoresces with a strong bluish color is frequently mixed with other phosphors, which fluoresce in the green or toward the red end of the spectrum, and the resultant mixture will fluoresce with substantially white light.

It is also known, in this art, that pure single phosphors, such as zinc sulfide, do not fluoresce as actively in their pure condition as they do when activated by a small percentage of one or more of certain other elements. It has been described by others how small traces of such elements as silver, gold, copper, beryllium, manganese, and other substances can be used to increase the luminescence (at certain wave lengths) obtained from a fluorescent body, such as a cathode ray tube screen, for a predetermined value of electrical excitation. It is likewise known that use of such "activators" results in substantial changes in the characteristic spectral responses. For example, zinc sulfide screens activated with silver sometimes have a high response in the green-yellow region. While such a response may be useful for certain purposes, it deleteriously affects the utility of the screens for the production of white light. This response is particularly objectionable when the fluorescent bodies are used as screens in television cathode ray tubes, since the television images appear greenish or yellowish, rather than being displayed in the desired black and white.

I have discovered that the aforesaid undesirable variations in spectral response are caused, to a large extent, by variations in the quantities and types of impurities present in the chemicals and

2

vessels as well as in the water used in the manufacturing process.

It is, therefore, an additional important object of this invention to provide a process characterized in that screens manufactured in accordance therewith result uniformly in production, without exhibiting the aforesaid wide variations in spectral response.

The foregoing, together with other objects and features characteristic of the invention, may be completely understood from a consideration of the following description, taken in the light of the accompanying drawing, in which:

Figure 1 is a graphical representation of the spectral response characteristic of several different cathode ray tube screens, one comprising silver-activated zinc sulfide, and another manganese-activated zinc beryllium silicate; and,

Figure 2 represents the optimum desired response characteristic, that is, the emission of white light, and indicates the deleterious changes or departures which are occasioned by the presence of copper activation, in an otherwise satisfactory screen.

As indicated above, it is known to widen the response band, and to approach the white light condition, by using two or more phosphors, for example, by using silver-activated zinc sulfide and manganese-activated zinc beryllium silicate.

First making reference to Figure 2, curve A is representative of the optimum results desired when several phosphors are used. As will be understood, the line designated A corresponds to the emission of white light. In Figure 2 wave lengths, as abscissa, are plotted against luminosity—relative to white—as ordinates.

In practice the results obtained, prior to the present invention, frequently approximated the results represented by curve B, the luminosity—relative to white—being objectionably high in the green-yellow portion of the spectrum with the result that the light emitted by the screen appeared greenish or yellowish, rather than white. As will now be understood such departures from the desired optimum condition are occasioned by the presence of undesired copper activation, and the cause and cure for the difficulty will become more apparent in what follows.

Prior to a detailed consideration of the process of the present invention, it is advantageous to

consider the manner in which cathode ray tube screens are commonly made. Accordingly, there is now presented, by way of example, an outline of a process commonly used for settling tube screens. This basic process yields good results, when modified in the light of the teachings of the present invention. As indicated above, the manner in which the basic process is thus modified will become clear hereinafter.

The basic process which I have used for settling tube screens, consists of agitating the silver-activated zinc sulfide and the manganese-activated zinc beryllium silicate (or the other phosphor combinations employed) in a solution including sodium sulfate, lithium hydroxide, potassium silicate and water. The resultant mixture, after being thoroughly agitated, is introduced into a glass blank of a cathode ray tube supported in such a position that the screen is in a horizontal plane, care being taken to prevent splashing of the sides of the blank. The particles suspended in the solution are then permitted to settle out on the screen surface. After the settling has been permitted to proceed for a predetermined length of time—dependent upon the particle size selected, the specific gravity of the overall mixture and the like—the remaining liquid is drained off either by the use of a siphon or by the decanting method, both of which will be well understood by one familiar with the art to which the invention pertains.

The screen formed by the aforesaid deposition process is then baked, in order to cause it to adhere firmly to the inside surface of the glass face of the tube. Following the baking process, the electron gun and other electrical components of the cathode ray tube are sealed into the glass blank. After the assembly is completed, the tube is evacuated and, during the evacuation process, the entire structure is again baked at a temperature sufficiently high to cause gases which may be occluded in the component parts to be released while the structure is still connected to the vacuum manifold.

I have found that this baking operation results, at times, in a shift of the color response of the screen. Experimentation has demonstrated that a large part of this shift in response, particularly when silver-activated phosphor is included, is due to the presence of varying amounts of impurity components that operate as activators. The principal offender among these impurities I found to be copper, which may be present in a variety of different forms. For example, impurities may be present as copper oxide, copper hydroxide, copper carbonate or copper sulfide.

The primary feature of this invention resides in the use of a scavenging agent in the liquid from which the phosphor is settled, which agent operates in such manner as to insure that copper impurities are held in soluble form. Substantially all such impurities may then be readily removed when the remaining liquid is removed by siphoning, decantation, or by any desired method employed for this purpose.

The presence of copper impurities may result from a number of different causes. I have found that, not infrequently, extremely small but deleterious quantities of copper impurities are present in the water, or in the sodium sulfate or other chemicals used in the preparation of the settling liquid. Traces of copper may also be present in the apparatus used. Similarly, the phosphors themselves, such as the silver-activated zinc sulfide and the manganese-activated zinc beryllium

silicate, which are preferably utilized, often contain, as contamination, a small percentage of copper. Phosphors which were recently used in the preparation of cathode ray screens in accordance with the present invention were found to contain small percentages of copper.

As indicated above, and again making particular reference to the drawing, the spectral response characteristics frequently show an excessive response in the green-yellow region.

In Figure 1, curve C represents the spectral response characteristic of pure silver-activated zinc sulfide, wave length being plotted against relative luminosity, in this figure. Due to the presence of the aforementioned traces of copper impurities, the response more commonly achieved with presumably pure silver-activated zinc sulfide approximates the response graphically represented by curve D. Curve E is indicative of the response characteristic of a representative screen consisting of manganese-activated zinc beryllium silicate only.

As set forth, supra, and in the preferred aspect of the invention, it is desired to compose a screen of both silver-activated zinc sulfide and manganese-activated zinc beryllium silicate. While these phosphors may be deposited separately, best results are achieved when both phosphors are settled-out of a single suspension. Prior to the present invention such mixtures did not consistently result in the emission of substantially white light. When the two phosphors indicated are mixed, the presence of the copper impurities, which caused the departure from the desired response characteristic (compare curves C and D, Figure 1), results in a curve of the type represented at B in Figure 2, rather than the desired characteristic depicted at A, in that figure.

Prior to the present invention such mixtures did not consistently result in the emission of substantially white light. Thus, such double phosphor screens, when contaminated with copper impurities, tend to fluoresce too strongly in the green-yellow portion of the spectrum.

In particular accordance with the present invention, the copper impurities are maintained in soluble form by the introduction, into the liquid suspension of phosphor, of a scavenging agent which holds the copper impurities in soluble form and makes it possible to remove them at the time of removal of the remaining liquid, and prior to the above-described baking.

I have found that components including a cyanide radical should be used as the scavenging agent, and, more particularly, that the use of potassium or sodium cyanide yields good results. The alkali cyanides, as a class, will yield satisfactory results as the scavenging agent, and in general, any cyanide may be used which will result in the formation—in the presence of the copper impurities—of a soluble copper-cyanide complex, providing that it yields less copper on ionizing than is required to form insoluble copper sulfide.

The amount of the scavenging substances to be added is dependent upon the quantities of copper impurities present. In practice it has proved that the addition of potassium or sodium cyanide, ranging in amount from about one-tenth percent to about one-half percent of the suspension liquid, by weight, achieved good results when commercially available phosphors were employed.

The scavenging agent, when added to the settling liquid at room temperature, reacts with the copper components, whether they be in soluble or insoluble form, forming soluble potassium cupro-

cyanide,  $K_3 Cu (CN)_4$ , which is the potassium salt of the complex anion  $Cu (CN)_4^{4-}$ . This anion shows extremely low ionization into  $Cu^+$  and  $CN^-$ .

The operation of and necessity for the scavenging agent will be better understood when it is borne in mind that the zinc sulfide phosphor, when suspended in water, undergoes a hydrolysis and, to a small extent, ionizes into zinc hydroxide and hydrogen sulfide. Copper in any of the simple compounds listed above would be precipitated as copper sulfide by the hydrogen sulfide. Copper held in solution as potassium cuprocyanide is not precipitated by hydrogen sulfide. This is the case because of the fact that the concentration of copper ions resulting from ionization of the soluble potassium cuprocyanide, is not sufficient to exceed the copper ion concentration (expressed in the solubility product of cuprous sulfide) required to cause precipitation of the slightly soluble copper sulfide.

Alkali cyanides dissolve copper oxide, copper hydroxide, copper carbonate, copper sulfide, etc., which substances change to soluble alkali cuprocyanides, rather rapidly. In these solutions, the concentration of the copper ion, as mentioned above, is so low that any hydrogen sulfide present forms insufficient cupric sulfide to be precipitated under these conditions.

I have found that the purposes of the present invention are best served when the hydrogen ion concentration of the settling solution lies in the range between pH 10.0 and pH 11.5. By keeping the hydrogen ion concentration in this range, and by having potassium or sodium cyanide present in the solution, substantially all of the copper impurities may be eliminated, as the screen settles out.

It is to be understood that the invention in its broader aspect, is not limited to the use of sodium or potassium cyanide. As indicated above other scavenging agents may be used to cause the copper impurities to be dissolved and held in solution as soluble complexes, rather than permitting them to settle with the other material, to the screen surface.

Further, it is to be understood that by the process of the present invention copper impurities (soluble or insoluble) are removed, whether they be originally introduced with the water, present in the apparatus, included with the phosphor, or present in the other chemical constituents used. The appended claims are to be understood with this in mind.

I claim:

1. In a process for settling phosphor out of a liquid suspension of said phosphor, which liquid suspension contains traces of copper impurities in normally insoluble form, the improvement which consists in utilizing a soluble alkali cyanide dissolved in the liquid of said suspension and effective to convert the copper impurities into soluble cuprocyanide complexes, and removing the supernatant liquid and the soluble complexes included therein.

2. In a process for settling phosphor out of a liquid suspension of said phosphor, which liquid suspension contains traces of copper impurities in normally insoluble form, the improvement which consists in utilizing sodium cyanide dissolved in the liquid of said suspension and effective to convert the copper impurities into soluble cuprocyanide complexes, and removing the supernatant liquid and the soluble complexes included therein.

3. In a process for settling phosphor out of a

liquid suspension of said phosphor, which liquid suspension contains traces of copper impurities in normally insoluble form, the improvement which consists in utilizing potassium cyanide dissolved in the liquid of said suspension and effective to convert the copper impurities into soluble cuprocyanide complexes, and removing the supernatant liquid and the soluble complexes included therein.

10. 4. In a process for settling phosphor, including silver-activated zinc sulphide, out of a liquid suspension of said phosphor, which liquid suspension contains traces of copper impurities in normally insoluble form, the improvement which

15 consists in utilizing a soluble alkali cyanide dissolved in the liquid of said suspension and effective to convert the copper impurities into soluble cuprocyanide complexes, and removing the supernatant liquid and the soluble complexes included therein.

20 5. In a process for settling phosphor, including silver-activated zinc sulphide, out of a liquid suspension of said phosphor, which liquid suspension contains traces of copper impurities in normally insoluble form, the improvement which

25 consists in utilizing sodium cyanide dissolved in the liquid of said suspension and effective to convert the copper impurities into soluble cuprocyanide complexes, and removing the supernatant liquid and the soluble complexes included therein.

30 6. In a process for settling phosphor, including silver-activated zinc sulphide, out of a liquid suspension of said phosphor, which liquid suspension contains traces of copper impurities in normally insoluble form, the improvement which

35 consists in utilizing potassium cyanide dissolved in the liquid of said suspension and effective to convert the copper impurities into soluble cuprocyanide complexes, and removing the supernatant liquid and the soluble complexes included therein.

40 7. A process in accordance with claim 4, and further characterized in that the hydrogen ion concentration of the liquid suspension is maintained in the range between pH 10.0 and pH 11.5.

45 8. In the art of producing fluorescent screens, the steps which comprise: providing a settling liquid including sodium sulphate, lithium hydroxide, potassium silicate and water; introducing silver-activated zinc sulphide and manganese-activated zinc beryllium silicate into said liquid; agitating the resultant mixture to cause said silver-activated zinc sulphide and said man-

50 ganese-activated zinc beryllium silicate to be suspended in said liquid; including in the liquid a soluble alkali cyanide to convert any copper impurities, which may be present, into soluble cuprocyanide complexes; and removing the supernatant liquid and the soluble complexes included therein.

55 9. A process in accordance with claim 8, and further characterized in that said soluble alkali cyanide is present in amount ranging from about one-tenth percent to about one-half percent of the suspension liquid, by weight.

60 10. In the art of producing fluorescent screens, the steps which comprise: providing an aqueous suspension of phosphor, said suspension containing traces of copper impurities in normally insoluble form; and utilizing a soluble alkali cyanide, dissolved in the suspension liquid, to bring the copper impurities into solution as soluble cuprocyanide complexes.

65 11. In the art of producing fluorescent screens,

the steps which comprise: providing an aqueous suspension of silver-activated zinc sulphide, said suspension containing traces of copper impurities in normally insoluble form; and utilizing a soluble alkali cyanide, dissolved in the suspension liquid, to bring the copper impurities into solution as soluble cuprocyanide complexes.

JOHN J. GEOGHEGAN.

REFERENCES CITED

The following references are of record in the file of this patent:

UNITED STATES PATENTS

| Number    | Name     | Date          |
|-----------|----------|---------------|
| 2,075,399 | Levy     | Mar. 30, 1937 |
| 2,219,929 | Kaufmann | Oct. 29, 1940 |

OTHER REFERENCES

Transactions of Illum. Eng. Soc., May 1939, article by Marsden et al., vol. 34, No. 5, pp. 509, 510, 512 and 513.

Mellor's Modern Inorganic Chemistry, 1939, pp. 594 and 595.